

**1**

2,753,274

**BITUMINOUS COMPOSITION**

Mathew L. Kalinowski, Chicago, Lowell T. Crews, Homewood, and John A. Bolt, Chicago, Ill., assignors to Standard Oil Company, Chicago, Ill., a corporation of Indiana

No Drawing. Application May 27, 1952,  
Serial No. 290,324

16 Claims. (Cl. 106—273)

The present invention is directed to improvements in bitumen compositions, and particularly to improvements in mineral aggregate coating compositions, and more particularly relates to bitumen compositions having improved adherence to damp or wet mineral aggregates.

Residual oils and/or bituminous materials used in the preparation of pavements and roads do not coat and adhere well to mineral aggregates unless the aggregate is substantially dry, and for this reason, in conventional pavements or road construction practice, it is customary to dry the mineral aggregate by suitable well known methods. Furthermore, water entering the road or pavement during service may have a detrimental effect in that it may displace the oil or bitumen from the surface of the aggregate and thus diminish the bonding effect of the oil and/or bitumen. This materially shortens the life of the road or pavement requiring frequent repairs and is, therefore, uneconomical.

Mineral aggregates employed in road or pavement construction range in character from hydrophilic to hydrophobic. In general, siliceous and acidic minerals, such as sands and gravels, tend to be hydrophobic, while calcareous, alkaline minerals, such as limestone, tend to be hydrophilic. It has been observed that the mineral aggregates appear to have a greater attraction for water than for oil or bitumen and that it is difficult to obtain, by conventional methods, complete or satisfactory coating of aggregates by oil or bitumen when water is present. Furthermore, even though satisfactory coating is obtained by using dry aggregate, the oil or bitumen tends to be displaced if water enters the pavement or road.

It is known that the coating of damp or wet mineral aggregates by oil or bitumen may be effected and the resistance of the coating to displacement or stripping by water improved by treating the aggregate with small amounts of a water-soluble soap of a fatty acid in conjunction with a water-soluble salt of a polyvalent heavy metal or "activator." For optimum results with these reagents, the relative amounts of the two reagents must be carefully adjusted. Thus, when a divalent heavy metal is used as activator, the amount of soap used should be substantially one mole per mole of activator; with a trivalent metal, between one and two moles of soap per mole of activator. Use of larger amounts of soap than this diminishes the effect obtained, and this diminution of effect increases with excess of soap over the proportions given until, when the amount of soap becomes equivalent to the activator, i. e., two moles of soap per mole of divalent metal or three per mole of trivalent metal, the beneficial effect of the reagent substantially disappears.

The above method has the disadvantage that the relative amounts of soap and polyvalent heavy metal activator are critical and must be carefully adjusted for optimum results. Use of an excess of soap over the optimum amount diminishes rather than enhances the effect obtained; the use of excess heavy metal to avoid the danger of excess soap is not harmful but increases the cost. Furthermore, the two reagents must be weighed or measured out and added to each batch, as neither is soluble in the oil or bitumen; while this disadvantage may be partially overcome under favorable conditions by using, in place of the soap, a fatty acid dissolved in the

**2**

oil or bitumen, this expedient is effective only under favorable conditions of low moisture content of the aggregate, adequate and efficient mixing, etc. Under conditions which are not at all severe, such as appreciable amounts of water and/or facilities for only moderately efficient mixing, fatty acids appear not to be sufficiently soluble in water to reach and react with the heavy metal ion to the required extent, and if added directly to the mixture or dissolved in the oil or bitumen, are practical-  
ly without effect.

Another important disadvantage of the above method is that a heavy polyvalent metal salt must be used with the soap. Furthermore, it has been found that while some limestones appear capable of adsorbing or reacting with polyvalent heavy metal ions and accordingly respond to some degree to the above method, a great many others do not, and with these it is difficult or impossible to obtain a good coating by the above method. Also, since the foregoing method is not in general satisfactory with limestone, a great many natural mixed aggregates such as gravels containing both siliceous and calcareous particles will have only a portion of the particles coated.

In addition to the use of polyvalent fatty acid soaps in bitumens as mineral aggregate coating agents, certain organic nitrogen compounds, such as those obtained by reacting a polyamine with a fatty acid under conditions to form essentially amides, have been used for this purpose. However, although the amide-type asphalt additives are effective coating agents for acidic mineral aggregates, such as sands and gravels, they are ineffective on alkaline mineral aggregates, such as limestone.

It is an object of the present invention to provide a bituminous material having improved coating properties. It is also an object of the present invention to provide an oil or bitumen composition which will adhere to wetted acidic and alkaline mineral aggregates. Another object of the present invention is to provide a coating composition for acidic and alkaline mineral aggregates which will not be stripped therefrom by aqueous liquids. Still another object of the invention is to provide a coating composition for acidic and alkaline mineral aggregates which can be applied without the necessity of drying the mineral aggregate, and which will adhere thereto even in a wet condition. Another object of the invention is to provide a method of preventing stripping of the coating composition from acidic and alkaline mineral aggregates by water after the road and/or pavement is constructed. A further object of the invention is to provide a method of promoting the adherence of oil bituminous materials to siliceous and limestone aggregates without the necessity of drying the same. Other objects and advantages of the invention will become apparent as description thereof proceeds.

In accordance with the present invention, bitumens, such as for example, road oils and asphalts having improved mineral aggregate coating properties, especially with respect to wet acidic and alkaline mineral aggregates, are obtained by incorporating in such bitumens from about 0.25% to about 5%, and preferably from about 0.5% to about 3%, by volume, based on the bitumen, of the oil-soluble product obtained by reacting an aliphatic polyamine with the propane-insoluble fraction obtained in the propane extraction of crude fatty materials, such as animal, marine and vegetable fats, fatty oils or fatty acids split therefrom, under conditions which avoid the formation of amides so that a product essentially free of amido groups is obtained. Since amidation of amine soaps is brought about by the loss of water at high temperatures, the reaction of the aliphatic polyamine with the aforementioned propane-insoluble fraction is carried out at temperatures below about 265° F., preferably below

about 240° F., and more preferably at temperatures of from about 180° F. to about 225° F.

The propane-insoluble fraction obtained in the propane extraction of crude fatty materials of the type above described contains, in addition to fats and fatty acids, esters of fatty acids and sterols. These propane-insoluble fractions which are obtained as residue of the order of about 0.2% to about 10%, by weight, contain most of the color bodies which are present in the crude fatty materials, and because of their very dark color, are referred to in commerce as "Ebony fats." The properties of representative samples of the propane insoluble residues obtained from animal fats and from vegetable oils, on a water-free basis, are approximately as follows:

| Property                                   | Residue from Animal Fat | Residue from Vegetable Oil |
|--------------------------------------------|-------------------------|----------------------------|
| Viscosity, Seconds Saybolt at 100° F.      | 6,500                   | 930                        |
| Viscosity, Seconds Saybolt at 130° F.      | 1,860                   | 430                        |
| Viscosity, Seconds Saybolt at 210° F.      | 300                     | 100                        |
| Ash, Weight.....percent.....               | 1.3                     | .06                        |
| A. P. I. Gravity.....degrees.....          | 10                      | 16                         |
| Acidity A. S. T. M. (D-664) Mg. KOH/gm.    | 41                      | 63                         |
| Pentane Insoluble, Weight.....percent..... | 2.6                     | 4.2                        |
| Benzene Insoluble, Weight.....percent..... | 7                       | 1.0                        |
| Saponification Number.....                 | 190                     | 170                        |
| Fatty Acid.....                            | 20                      | 31                         |
| Iodine Number.....                         | 58                      | 106                        |

The above properties are, of course, merely illustrative, and it should be understood that both the amount and the property of the propane-insoluble residues depend upon the nature of the crude fatty material extracted, and upon the particular conditions employed in effecting the extracted fractionation. The term "crude" as used herein means that the color bodies and other materials, insoluble in 6 to 30 volumes of the propane at about 140° F. to about 190° F. have not been removed regardless of whether or not the fatty material has been destearinized.

The method of fractionating the animal, marine and vegetable fatty materials with propane to obtain "Ebony fat" is well known to those skilled in the art and one example thereof is commonly referred to as the "Solexol process," currently and commercially used and described in "Industrial and Engineering Chemistry" of February 1949, page 280. The system for effecting such extractive fractionation is described in detail in U. S. 2,505,338 and U. S. 2,521,234. For most crude animal fats, marine oils and vegetable oils, and similar fatty materials, including acids split from such fats, the fractionation conditions are employed which give a propane-insoluble residue of about 1%, i. e., about 0.2% to about 2%, although in some cases such residues may be as large as 5% or even 10%.

The amine reactant employed in preparing the additive of the present invention is an aliphatic polyamine, particularly an alkylene polyamine containing at least two primary amino nitrogen atoms. Examples of alkylene polyamines suitable for the herein-described purpose are ethylene diamine, propylene diamine, diethylene triamine, diamylene triamine, triethylene tetramine, tripropylene tetramine, diethylenepropylene tetramine, tetraethylene pentamine, tetrabutylene pentamine, diethylenedipropylene pentamine, butylene diamine, dihexylene triamine, and the like, or mixtures thereof. For example, a suitable polyamine product is a crude diethylene triamine containing minor amounts of ethylene diamine and triethylene tetramine. Other suitable polyamines include those having the general formula  $RNH(CH_2)_3NH_2$  in which R is preferably a  $C_{10}$  to  $C_{18}$  aliphatic chain, and which are obtained by condensing the suitable amine with acrylonitrile and hydrogenating to the corresponding diamine. Commercially available polyamines of this type are those marketed by Armour and Company as "Duomeens," which are prepared by the condensation of a dodecyl (Coco) amine or an octadecyl (tallow) amine

with acrylonitrile, followed by hydrogenation to the corresponding diamine product; these products are marketed as "Duomeen C" and "Duomeen T," respectively.

In the preparation of the "Ebony fat" and polyamine reaction product, it is preferable, although not essential, that the "Ebony fat" be first dehydrated to obtain an essentially water-free product, or a product having not more than 0.5% water. This can be readily accomplished by diluting the "Ebony fat" with from about 10% to about 50% of a suitable hydrocarbon solvent, preferably a solvent rich in aromatic hydrocarbons, and by heating the diluted mixture at a temperature of about 210° F. to 290° F. while stirring and/or blowing with air or other suitable gaseous medium until the water content has been reduced to the desired value. If the "Ebony fat" contains an undesirable amount of contaminants, they can be removed by permitting the hot dehydrated solution to settle, and decanting the diluted solution of purified "Ebony fat." If desired, the diluent may be removed from the dehydrated "Ebony fat" by suitable means, such as by distillation under vacuum; however, we prefer to react the diluted "Ebony fat" with the polyamine.

Aromatic-rich hydrocarbon solvents suitable for this purpose are preferably those having boiling points above about 220° F. at atmospheric pressure and includes mono-nuclear aromatic hydrocarbons or condensed ring aromatics, such as naphthalenes and mixtures of the higher boiling mono-nuclear aromatic hydrocarbons and poly-nuclear aromatic hydrocarbons.

A preferred source of mixed aromatic hydrocarbons suitable for the purpose, is a light catalytic cycle stock obtained from a powdered or a fluid-type catalytic-type hydrocarbon cracking operation in which gas oil or heavier hydrocarbons are cracked at a temperature of 800° F. to 1050° F., under a pressure of about atmosphere to 50 pounds per square inch, in the presence of suitable fluid or powdered catalyst, such as for example, silica-alumina, silica magnesia, and other well-known cracking catalysts. A method of conducting a fluidized cracking operation is described in U. S. 2,341,193 issued to Fred W. Scheineman, February 8, 1944. Fractions from the process heavier than gasoline, depending upon their boiling range, are commonly referred to as light catalytic cycle stock, heavy catalytic cycle stock and catalytic recycle resid, which usually are cycled to cracking. A light catalytic cycle stock particularly well suited as a diluent for the dehydration of the "Ebony fat" is a fraction having an aromatic content of at least about 40% and a distillation range between about 425° F. and about 560° F. A typical analysis of a suitable light catalytic cycle stock shows the material to be composed substantially of about 10% normal  $C_{12}$  to  $C_{20}$  paraffins, about 45% of other paraffins, and naphthenes, about 5% mono-nuclear aromatics, which are mainly mono- to hexa-alkylated benzenes, and about 40% polynuclear aromatics, which are mainly alkyl naphthalenes, largely methylated naphthalenes. While we prefer to use a light catalytic cycle stock of the type described, hydrocarbon fractions from other catalytic conversion processes or thermal hydrocarbon conversion processes are suitable, provided they have an aromatic content of at least about 20%, and a distillation range of above about 220° F.

The dehydrated "Ebony fat" preferably, but not necessarily, in solution in the light catalytic cycle stock or other suitable diluent, is reacted with the polyamine in the ratio of from about 20:1 to about 5:1, and preferably in a ratio of from about 12:1 "Ebony fat" to the polyamine, at a temperature below about 265° F., and preferably of from about 180° F. to about 225° F., for not more than about one hour, and the temperature then reduced as rapidly as possible to about 170° F., or lower. By conducting the reaction in the manner herein described, and maintaining the finished product, until ready for use, at a temperature below about 150° F., and pref-

erably below about 140° F., an efficient stable coating agent essentially free of amido groups is obtained.

The preparation of polyamine-“Ebony fat” reaction products is illustrated by the following examples:

#### EXAMPLE I

161 pounds of “Ebony fat” were mixed with 79 pounds of light catalytic cycle stock and dehydrated at a temperature of 280° F. to 295° F. for about one and three-quarters hours while blowing air through the mixture. The temperature of the mixture was then lowered to 210° F., 12 pounds of ethylene diamine added, and the mixture heated and cooled according to the following schedule:

10 minutes at 210° F. to 240° F.;  
10 minutes at 240° F. to 260° F.;  
10 minutes at 260° F. to 265° F.;  
20 minutes at 265° F., and  
25 minutes to cool from 265° F. to 175° F.

A yield of about 248 pounds of the reaction product in light catalytic cycle stock solution containing about 66½% of the active additive was obtained.

#### EXAMPLE II

160 pounds of “Ebony fat” was mixed with 80 pounds of light catalytic cycle stock and dehydrated at 255° F. to 295° F. for four and one-quarter hours while blowing air through the mixture. To the dehydrated “Ebony fat” were added 15 pounds of triethylene tetramine (66%) and the mixture stirred at 240° F. to 265° F. for one hour. The temperature was then lowered to 220° F. for one hour and then rapidly reduced to 175° F.

#### EXAMPLE III

300 grams of “Ebony fat”, dehydrated as in Example II, were reacted with 28 grams of tetraethylene pentamine at a temperature of about 225° F. for about one hour, and then rapidly cooled to about 170° F.

#### EXAMPLE IV

A dehydrated mixture of 300 grams of “Ebony fat” in 150 grams light catalytic cycle stock was reacted with 20 grams of propylene diamine under conditions given in Example III.

#### EXAMPLE V

A solution of 2500 gallons of “Ebony fat” in 2500 gallons of light catalytic cycle stock was heated to about 240° F., and blown with air, for about four hours, until the water content was reduced to 0.15%. At a temperature of 230° F., 300 gallons of triethylene tetramine were added, and the reaction was allowed to proceed for one-half hour. Cooling water was then turned on, the mixture was cooled to 120° F., and was then pumped to finished additive storage.

#### EXAMPLE VI

100 grams of “Ebony fat” and 120 grams of light catalytic cycle stock were mixed and heated to 210° F.-250° F., while air blowing until the mixture was substantially anhydrous. Twenty grams of “Duomeen T” were added and heated at 230° F. to 250° F. for one-half hour and then cooled.

#### EXAMPLE VII

The corresponding reaction product of “Ebony fat” and “Duomeen C” was prepared as the corresponding “Duomeen T” product in Example VI.

#### EXAMPLE VIII

A solution of 3000 gallons of “Ebony fat” and 2000 gallons of light catalytic cycle stock was heated to about 240° F. and blown with air for about four hours to dehydrate the “Ebony fat” from a water content of 2.5% to a water content of 0.2%. To the dehydrated “Ebony fat” solution were added 225 gallons of ethylene

5 diamine (76%) at a temperature of 240° F.-245° F. Twenty minutes after all of the ethylene diamine was added, cooling water was turned on and the reaction mixture cooled in three hours time to 170° F. Cooling was continued to a temperature of 120° F. and the reaction product filled into barrels at 90° F.

10 While we have not been able to definitely determine the composition of the “Ebony fat”-polyamine reaction product, we believe the reaction comprises essentially the amine soaps of the fatty acids contained in the “Ebony fat,” together with unreacted esters and alcohols, i.e., sterols.

15 The asphalt component of the herein-described composition may be any bitumen which is useful for the coating of mineral aggregates used in the making of roads, highways, etc., or for the coating of other materials or surfaces where a water-resistant bond between the surface and the asphalt is advantageous or necessary. The term “asphalt” as employed herein is intended to be synonymous with bitumen and to cover a liquid, semi-solid, or solid plastic bituminous material of the type employed in making or surfacing of highways and/or pavements, caulking agents, sealing compounds, water impervious paints, roofing materials, etc. Such asphalt or bituminous materials are mixtures of hydrocarbons of natural or pyrogenic origin, and are usually derived from petroleum or coal but may occur as such in nature. Asphalts may be derived as distillation resids or cracking resids with or without oxidation by air-blowing or by catalytic oxidation. A specific example of a liquid asphalt of the type commonly employed in the preparation of highways, etc. is a petroleum residuum fluxed with a light aromatic diluent boiling in the range of 400° F. to 700° F. to give a cutback product of the following 20 specifications:

|                             | Cutback asphalt       |
|-----------------------------|-----------------------|
| Flash, °F. (T. O. C.)       | <sup>1</sup> NLT 150  |
| Viscosity, furol at 140° F. | 100-200               |
| ASTM distillation:          |                       |
| Per cent off at 437° F.     | <sup>2</sup> NMT 10.0 |
| Per cent off at 500° F.     | 15-55                 |
| Per cent off at 600° F.     | 60.87                 |
| Residue at 680° F.          | NLT 67.0              |

#### Tests on distillation:

|                                     |          |
|-------------------------------------|----------|
| Residue:                            |          |
| ASTM penetration at 77° F.          | 120-300  |
| ASTM ductility at 77° F.            | NLT 100  |
| Sol. in CCl <sub>4</sub> , per cent | NLT 99.5 |
| Oiliensis spot test                 | Negative |

<sup>1</sup> “Not less than”  
<sup>2</sup> “Not more than”

Normally solid paving asphalts of the 40 to 200 penetration grades commonly used in road building fall within the following specifications:

|                                                                   |                            |
|-------------------------------------------------------------------|----------------------------|
| Penetration at 77° F.                                             | 40-200.                    |
| ASTM ductility at 77° F.                                          | Not less than 100.         |
| Oiliensis spot test                                               | Negative.                  |
| Solubility in CCl <sub>4</sub> , percent                          | Not less than 99.5.        |
| Specific gravity at 60° F.                                        | Not less than 0.990-1.000. |
| Flash, °F. (C. O. C.)                                             | Not less than 475.         |
| Loss on heating 50 grams for 5 hours at 325° F., percent          | Not more than 0.5.         |
| Penetration of residue at 77° F., percent of original penetration | Not less than 70-75.       |

The effectiveness of the herein-described “Ebony Fat”-polyamine reaction products in enhancing the adhesion of asphalts to wet mineral aggregates is determined by subjecting blends of asphalts and the described reaction products to one or more of the following tests:

#### A. Modified Colorado coating tests

20 grams of Ottawa sand or 20 grams of a 20 to 35 mesh limestone are weighed into a 2 oz. container and

covered with one-half inch of distilled water. One gram of the additive-containing asphalt is floated on the water, the mixture then shaken for thirty seconds, and the extent of coating determined by visual inspection; the results are expressed as "Percent Coated."

B. *Wyoming stripping test*

Approximately 25 g. of Lander chips, all passing the  $\frac{3}{8}$  inch sieve and retained on the No. 4 sieve, is mixed by hand with 1.0 g. of fortified asphalt until the best possible coating is obtained. The mix is placed in an oven at 140° F. for 18 to 24 hours after which it is thoroughly remixed and is allowed to cool to room temperature. The sample is then immersed in distilled water at a temperature of 120° F., and is maintained at this temperature for a period of 24 hours. At the end of this period the area of the aggregate remaining coated is determined visually while the sample is still under water. Any thin or translucent areas are considered to be coated. The Wyoming Highway Department requires that 80% or greater coating be retained in this test.

C. *Hot settling test*

300 grams of asphalt containing 2% of the additive are stored in a closed one pound tin container at 170° F. for twenty-four hours. At the end of this period the percent of sediment is determined gravimetrically. A value less than 2% is considered desirable. The asphalt-additive mixture after being stored at 170° F. for the 24-hour period is retested by the Colorado Coating Test (supra) for its ability to coat wet aggregates.

The data obtained by subjecting blends of a cutback asphalt of the above specification and various "Ebony Fat"-polyamine reaction products, prepared in the manner herein described, to one or more of the above-described tests are given in Table I.

TABLE I

| Additive       | Colorado Coating Test |                    | Wyoming Stripping Test, percent | Hot Settling Test |                  |                    |  |
|----------------|-----------------------|--------------------|---------------------------------|-------------------|------------------|--------------------|--|
|                | Sand, percent         | Limestone, percent |                                 | Sediment, percent | Colorado Coating |                    |  |
|                |                       |                    |                                 |                   | Sand, percent    | Limestone, percent |  |
| None (Control) | 0                     | 0                  | 10                              | 0.0               | 0                | 0                  |  |
| Control+1% A   | 95+                   | 80                 | 70                              | 0.0               | 100              | 90                 |  |
| Control+2% A   | 100                   | 90                 | 90                              | 0.0               | 100              | 90                 |  |
| Control+1% B   | 85-90                 | 90                 | 70                              | 0.8               | 95               | 90                 |  |
| Control+2% B   | 100                   | 90                 | 95                              | 0.8               | 95               | 90                 |  |
| Control+1% C   | 80                    | 80                 | 75                              | 0.0               | 100              | 90                 |  |
| Control+1% C   | 100                   | 90                 | 85                              | 0.0               | 100              | 90                 |  |
| Control+1% D   | 80                    | 80                 | 85                              | 0.0               | 100              | 90                 |  |
| Control+1% D   | 100                   | 85                 | 80                              | 0.0               | 100              | 90                 |  |
| Control+1% E   | 95+                   | 80                 | 85                              | 0.2               | 100              | 100                |  |
| Control+2% F   | 100                   | 100                | 100                             | 0.0               | 100              | 100                |  |
| Control+1% G   | 95                    | 5                  | 90                              | 0.0               | 90               | 5                  |  |
| Control+1% G   | 100                   | 10                 | 95                              | 0.0               | 100              | 10                 |  |
| Control+1% H   | 100                   | 90                 | 45                              | 0.0               | 100              | 10                 |  |
| Control+2% H   | 100                   | 100                | 95                              | 0.0               | 0                | 10                 |  |
| Control+1% K   | 100                   | 90                 | 75                              | 0.0               | 100              | 10                 |  |
| Control+2% K   | 100                   | 100                | 100                             | 0.1               | 10               | 15                 |  |

In Table I the various additives are identified as follows:

son, a commercial asphalt additive was subjected to the same test. The results obtained are tabulated in Table II.

TABLE II

| Storage Temperature   | 77° F.                   |      |            |      |            |      | 140° F.    |      |            |      |            |      | 170° F.    |      |            |      |            |      |
|-----------------------|--------------------------|------|------------|------|------------|------|------------|------|------------|------|------------|------|------------|------|------------|------|------------|------|
|                       | 0                        |      | 20         |      | 60         |      | 10         |      | 14         |      | 31         |      | 7          |      | 14         |      | 31         |      |
|                       | Percent Colorado Coating | Sand | Lime-stone | Sand | Lime-stone | Sand | Lime-stone | Sand | Lime-stone | Sand | Lime-stone | Sand | Lime-stone | Sand | Lime-stone | Sand | Lime-stone | Sand |
| Control (No Additive) | 0                        | 0    | 0          | 0    | 0          | 0    | 0          | 0    | 0          | 0    | 0          | 0    | 0          | 0    | 0          | 0    | 0          | 0    |
| Control+2% "B"        | 100                      | 95   | 100        | 95   | 100        | 95   | 100        | 95   | 100        | 90   | 80         | 90   | 90         | 85   | 70         | 90   | 90         | 90   |
| Control+0.5% "G"      | 100                      | 0    | 90         | 0    | 90         | 0    | 5          | 0    | 100        | 95   | 0          | 5    | 0          | 0    | 0          | 0    | 0          | 90   |

Additive "B"—Same as in Table I.

Additive "G"—Same commercial asphalt additive as in Table I.

"A." Reaction product of "Ebony fat" and ethylene diamine prepared as in Example VIII.

"B." Reaction product of "Ebony fat" and diethylene triamine prepared as in Example II.

"C." Reaction product of "Ebony fat" and "Duomeen T" prepared as in Example VI.

"D." Reaction product of "Ebony fat" and "Duomeen C" prepared as in Example VII.

"E." Reaction product of "Ebony fat" and tetraethylene pentamine prepared as in Example III.

"F." Reaction product of "Ebony fat" and propylene diamine prepared as in Example IV.

"G," "H," and "K." Commercial asphalt coating agents comprising essentially fatty acid - polyamine amides.

The data in Table I demonstrate the effectiveness of the "Ebony-fat"-polyamine reaction product, prepared in the manner herein-described, in maintaining asphalt coatings on both wet acidic and alkaline mineral aggregates. The data with respect to additives "G," "H" and "K," the above-described commercial asphalt coating agents, demonstrate the ineffectiveness of these products with respect to the coating of alkaline mineral aggregates, such as limestone and/or the heat instability of such additives.

The asphalt additives of the present invention exhibit exceptionally good stability with respect to resistance to coating degradation under typical storage temperatures ranging up to 170° F., as well as under typical field application temperatures of about 230° F.

The heat stability of the asphalt additives was determined by storing asphalts containing the additives of the present invention in glass jars at temperatures of 77° F., 140° F., and 170° F., for various periods and testing each sample after such test periods by the Colorado Coating Test (supra). For purposes of compari-

The heat stability of applicants' asphalt additive under typical storage temperature conditions and its superiority over the commercial amide product are clearly demonstrated by the data in Table II.

Since asphalts are applied at somewhat elevated temperatures up to about 230° F., it is important that such additive-containing asphalts show no degradation or loss in efficiency at such temperatures. The heat stability of applicant's herein described "Ebony fat"-polyamine reaction products at temperatures up to about 230° F., which is a typical temperatures at which asphalts are applied in road building or repair, is shown by the data in Table III. These data were obtained by storing additive-containing asphalt samples at a temperature of 230° F. for periods of time, and at stated intervals, testing such samples for their coating efficiency by the Colorado Coating Test, and the Wyoming Stripping Test (supra). The results obtained demonstrate that applicants' additives are heat stable at temperatures as high as 230° F. for as long as fifty-four hours. For comparative purposes, an asphalt containing the commercial product, hereinabove described, was also tested under the same conditions.

TABLE III

| Hours at 230° F.      | Colorado Coating |            |      |            |      |            |      |            | (Lander Chips) Wyoming Stripping |         |         |         |
|-----------------------|------------------|------------|------|------------|------|------------|------|------------|----------------------------------|---------|---------|---------|
|                       | 0                |            | 24   |            | 48   |            | 54   |            | 0                                |         | 24      |         |
|                       | Sand             | Lime-stone | Sand | Lime-stone | Sand | Lime-stone | Sand | Lime-stone | Percent                          | Percent | Percent | Percent |
| Control (No Additive) | 0                | 0          | 0    | 0          | 0    | 0          | 0    | 0          | 0                                | 0       | 0       | 0       |
| Control+2.0% "B"      | 100              | 85         | 95   | 85         | 95   | 85         | 90   | 85         | 95                               | 10      | 95      | 10      |
| Control+0.5% "G"      | 100              | 0          | 90   | 0          | 75   | 0          | 95   | 0          | 85                               | 80      | 40      | 70      |

Additive "B"—Same as in Table II.

Additive "G"—Same as in Table II.

The data of Table III show the heat stability of the asphalt additives of the herein described invention at typical application temperatures. The data also demonstrate the increased heat stability of the "Ebony fat" polyamine reaction products, essentially free of amides over that of a commercial product which is essentially an amide product.

Although the "Ebony fat"-polyamine reaction products are heat stable at temperatures as high as 230° F., and exhibit essentially no degradation with respect to coating and stripping efficiency, it is advisable to limit the blending and/or storage temperature for the fortified asphalts to temperatures not in excess of about 150° F., and preferably at temperatures not in excess of 140° F. Likewise, asphalts containing the herein-described asphalt additives should preferably be applied at temperatures not to exceed about 230° F.

While the present invention has been described by reference to specific embodiments thereof, these are given by way of illustration only, and the invention is not to be limited thereto but includes within its scope such modifications and variations as come within the spirit of the appended claims.

We claim:

1. A bitumen composition comprising a major proportion of bitumen from about 0.25% to about 5% of the oil-soluble reaction product of an alkylene polyamine, having from 2 to about 20 carbon atoms, and "Ebony fat" which "Ebony fat" is the propane-insoluble residue obtained in the solvent extraction of a crude fatty material selected from the class consisting of crude animal fats, fatty oils, and fatty acids, crude vegetable fats, fatty oils, and fatty acids, and mixtures thereof, with liquefied propane, said insoluble residue being insoluble in 6 to 30 volumes of propane at a temperature of from about 140° F. to about 190° F. and constituting from about 0.2% to about 10% of the crude fatty material from which said insoluble residue is extracted, said oil-soluble reaction product being essentially free of amido groups.

10 to about 10% of the crude fatty material from which said insoluble residue is extracted, said oil-soluble reaction product being essentially free of amido groups.

2. A bitumen composition as described in claim 1, in which the alkylene polyamine is an alkylene polyamine containing at least two primary amino nitrogen atoms.
3. A bitumen composition as described in claim 1, in which the alkylene polyamine is an alkylene diamine.
4. A bitumen composition as described in claim 1 in which the alkylene polyamine is ethylene diamine.
5. A bitumen composition as described in claim 1, in which the alkylene polyamine is diethylene triamine.
6. A bitumen composition as described in claim 1, in which the alkylene polyamine is a polyamine mixture comprising essentially diethylene triamine and minor amounts of ethylene diamine and triethylene tetramine.
7. A bitumen composition as described in claim 1, in which the alkylene polyamine is a trialkylene tetramine.
8. A bitumen composition as described in claim 1, in which the alkylene polyamine is triethylene tetramine.
9. A bitumen composition as described in claim 1, in which the alkylene polyamine has the general formula:



in which R is an aliphatic group containing from about 10 to about 18 carbon atoms.

10. A bitumen composition as described in claim 1 in which the crude fatty material is a crude animal fat.
11. A bitumen composition as described in claim 1 in which the crude fatty material is a crude vegetable oil.
12. A bitumen composition as described in claim 1 in which said oil-soluble reaction product is diluted with from about 10% to about 50% of an aromatic-rich hydrocarbon diluent having a boiling point above 220° F.
13. A bitumen composition as described in claim 1 in which the bitumen is a normally liquid bitumen.
14. A bitumen composition as described in claim 1 in which the bitumen is a normally solid paving asphalt.
15. A roadway construction material resistant to water stripping comprising mineral aggregates admixed with a coating composition comprising a major proportion of a normally liquid bitumen and from about 0.25% to about 5% of the oil-soluble reaction product of an alkylene polyamine, having from 2 to about 20 carbon atoms, and "Ebony fat" which "Ebony fat" is the propane-insoluble residue obtained in the solvent extraction of a crude fatty material selected from the class consisting of crude animal fats, fatty oils, and fatty acids, crude vegetable fats, fatty oils, and fatty acids, and mixtures thereof, with liquefied propane, said insoluble residue being insoluble in 6 to 30 volumes of propane at temperatures of from about 140° F. to about 190° F. and constituting from about 0.2% to about 10% of the crude fatty material from which said insoluble residue is extracted, said oil-soluble reaction product being essentially free of amido groups.
16. A composition described in claim 15 in which the normally liquid bitumen is a petroleum residuum.

**11****References Cited in the file of this patent****UNITED STATES PATENTS**

2,329,889 Ewing Sept. 21, 1943  
2,383,097 Watman Aug. 21, 1945  
2,436,599 Read et al. Feb. 24, 1948

2,534,713  
2,542,982

5 151,666

**12**

Hankins Dec. 19, 1950  
Bartleson et al. Feb. 27, 1951

**FOREIGN PATENTS**

Great Britain Oct. 7, 1920